



US006002322A

# United States Patent [19]

Krueger et al.

[11] Patent Number: 6,002,322

[45] Date of Patent: \*Dec. 14, 1999

## [54] CHIP PROTECTOR SURFACE-MOUNTED FUSE DEVICE

[75] Inventors: **David J. Krueger**, Arlington Heights; **Brian J. Bullock**, Elmhurst; **Honorio S. Luciano**, Elk Grove Village, all of Ill.[73] Assignee: **Littelfuse, Inc.**, Des Plaines, Ill.

[\*] Notice: This patent issued on a continued prosecution application filed under 37 CFR 1.53(d), and is subject to the twenty year patent term provisions of 35 U.S.C. 154(a)(2).

[21] Appl. No.: 09/072,964

[22] Filed: May 5, 1998

[51] Int. Cl.<sup>6</sup> ..... H01H 85/046; H01H 85/20; H01H 69/02

[52] U.S. Cl. ..... 337/297; 337/296; 430/311; 430/314; 29/623

[58] Field of Search ..... 337/152, 160, 337/227, 297, 296; 430/325, 327, 322, 323, 328-331, 313, 314, 315-318, 311; 29/623

## [56]

## References Cited

## U.S. PATENT DOCUMENTS

|           |         |                            |         |
|-----------|---------|----------------------------|---------|
| 3,629,036 | 12/1971 | Isaacson .....             | 156/241 |
| 4,069,076 | 1/1978  | Fickes .....               | 156/83  |
| 4,506,004 | 3/1985  | Sullivan .....             | 430/312 |
| 4,698,294 | 10/1987 | Lau et al. ....            | 430/325 |
| 5,213,945 | 5/1993  | Roos et al. ....           | 430/270 |
| 5,228,188 | 7/1993  | Badihi et al. ....         | 29/623  |
| 5,405,731 | 4/1995  | Chandrasekaran et al. .... | 430/260 |
| 5,552,757 | 9/1996  | Blecha et al. ....         | 337/297 |
| 5,601,905 | 2/1997  | Watanabe et al. ....       | 428/215 |
| 5,726,621 | 3/1998  | Whitney et al. ....        | 337/297 |

Primary Examiner—Donald Sparks

Assistant Examiner—Anatoly Vortman

Attorney, Agent, or Firm—Wallenstein &amp; Wagner, Ltd.

## [57]

## ABSTRACT

A thin film, surface-mounted fuse which comprises two material subassemblies. The first subassembly comprises a fusible link, its supporting substrate and terminal pads. The second subassembly comprises a protective, photoimageable layer which overlies the fusible link so as to provide protection from impacts and oxidation. The photoimageable layer is a low profile coating.

6 Claims, 4 Drawing Sheets



FIG. 1



FIG. 2



FIG. 3



FIG. 4



FIG. 5



FIG. 6



FIG. 7



FIG. 8



FIG. 9



FIG.10



FIG.11



FIG.12



# CHIP PROTECTOR SURFACE-MOUNTED FUSE DEVICE

## TECHNICAL FIELD

The invention relates generally to the use of photoimageable materials as conformal coatings for surface-mountable fuses. Such fuses are placed into and are used for the protection of the electrical circuit of a printed circuit board.

## BACKGROUND OF THE INVENTION

Printed circuit (PC) boards have found increasing application in electrical and electronic equipment of all kinds. The electrical circuits formed on these PC boards, like larger scale, conventional electrical circuits, need protection against electrical overloads. This protection is typically provided by subminiature fuses that are physically secured to the PC board.

One example of such a subminiature, surface-mounted fuse is disclosed in U.S. Pat. No. 5,166,656 ('656 patent). The fusible link of this surface-mounted fuse is disclosed as being covered with a three layer composite which includes a passivation layer, an insulating cover, and an epoxy layer to bond the passivation layer to the insulating cover. See '656 patent, column 6, lines 4-7. Typically, the passivation layer is either chemically vapor-deposited silica or a thick layer of printed glass. See '656 patent, column 3, lines 39-41. The insulating cover may be a glass cover. See '656 patent, column 4, lines 43-46.

Another prior art device is described in U.S. Pat. No. 5,552,757. In that invention, unlike the '656 patent, the fusible link is protected with only one, rather than three, layers. In the '757 patent, however, this one protective layer 56 is a polycarbonate adhesive or the like. This protective layer 56 extended substantially above the general borders of the surface-mount fuse shown in FIG. 12 of the '757 patent. As a result, the fuse shown in FIG. 12 of the '757 patent could only be placed on a circuit board with the protective layer 56 facing upwardly, away from the board.

## SUMMARY OF THE INVENTION

The invention is a thin film, surface-mounted fuse which comprises two material subassemblies. The first subassembly comprises a fusible link, its supporting substrate and terminal pads. The second subassembly comprises a protective, photoimageable layer which overlies the fusible link so as to provide protection from impacts and oxidation. The second subassembly in the present invention is a photoimageable material.

The photoimageable material can be applied as either a liquid or a solid. The liquid material is dried after application. The solid may be a film that is vacuum applied. Whether the photoimageable material is a liquid or a solid film, portions of the material are cured onto the substrate through photoexposure. Uncured or unexposed portions of the material are selectively removed from the substrate during a developing process. This process results in a targeted application of the photoimageable material.

Photolithographic, mechanical and laser processing techniques may be employed to create very small, intricate and complex fusible link geometries. This capability, when combined with the application of ultra thin photoimageable conformal coatings, enables these subminiature fuses to control the fusible area of the element and protect circuits passing microampere- and ampere-range currents.

## BRIEF DESCRIPTION OF THE DRAWINGS

FIG. 1 is a perspective view of a copper-plated, FR-4 epoxy sheet used to make a subminiature surface-mounted fuse in accordance with the invention.

FIG. 2 is a view of a portion of the sheet of FIG. 1, and taken along lines 2—2 of FIG. 1.

FIG. 3 is a perspective view of the FR-4 epoxy sheet of FIG. 1, but stripped of its copper plating, and with a plurality of slots, each having a width W and a length L, routed into separate quadrants of that sheet.

FIG. 4 is an enlarged, perspective view of a portion of the routed sheet of FIG. 3, but with a copper plating layer having been reapplied.

FIG. 5 is a top view of several portions of the flat, upward-facing surfaces of the replated copper sheet, after each of those portions were masked with a square panel of an ultraviolet (UV) light-opaque substance.

FIG. 6 is a perspective view of the reverse side of FIG. 5, but after the removal of a strip-like portion of copper plating from the replated sheet of FIG. 5.

FIG. 7 is a perspective view of the top-side 38 of the strip 26 of FIG. 6, and showing linear regions 40 defined by dotted lines.

FIG. 8 is a view of a single strip 26 after dipping into a copper plating bath and then a nickel plating bath, with the result that copper and nickel layers are deposited onto the base copper layer of the terminal pads.

FIG. 9 is a perspective view of the strip of FIG. 8, but prior to UV light curing, and showing a portion 50 at the center of fusible link 42 that is masked with a UV light-opaque substance.

FIG. 10 shows the strip of FIG. 9, but after immersion into a tin plating bath to create another layer over the copper and nickel layers, and after deposition of tin onto the central portion of the fusible link.

FIG. 11 shows the strip of FIG. 10, but with an added photoimageable layer placed onto the top of the strip 26.

FIG. 12 shows the individual fuse in accordance with the invention as it is finally made, and after a so-called dicing operation in which a diamond saw is used to cut the strips along parallel planes to form these individual surface-mountable fuses.

## DETAILED DESCRIPTION OF THE PREFERRED EMBODIMENT

While this invention may include any of several embodiments, the drawings describe one preferred embodiment. The disclosure does not limit the invention to the illustrated embodiment.

A preferred embodiment of the present invention is shown in FIG. 12. The thin film, surface-mounted fuse is a subminiature fuse used in a surface mount configuration on a PC board or on a thick film hybrid circuit. These fuses are typically known in the art as "A" case fuses. The standard industry size for these fuses is 125 mils. long by 60 mils. wide. Such fuses are designated, for shorthand purposes, as 1206 fuses. It will be understood, however, that the present invention can be used on all other standard sizes of such fuses, such as 1210, 0805, 0603 and 0402 fuses, as well as non-standard sizes.

In its broadest concept, the invention comprises two material subassemblies. As will be seen, the first subassembly includes the fuse element or fusible link 42, its supporting substrate or core 13, and terminal pads 34 and 36 for connecting the fuse 58 to the PC board. The second subassembly is a novel, photoimageable protective layer 56 which overlies the fusible link 42 and a substantial portion of the top portion of the fuse so as to provide protection from impacts which may occur during automated assembly, and protection from oxidation during use.

The first subassembly contains and supports two metal electrodes or pads and the fusible element, both of which are bonded to the substrate as a single continuous film. The pads are located on the bottom and sides of the substrate or core, while the fusible link is located at the top of the substrate or core.

As will be seen, in the preferred embodiment, pads are made up of several layers, including a base copper layer, a supplemental copper layer, a nickel layer and a tin layer. The base copper layer of the pads and the thin film fusible link are simultaneously deposited by (1) electrochemical processes, such as the plating described in the preferred embodiment below; or (2) by PVD. Such simultaneous deposition ensures a good conductive path between the fusible link and the terminal pads. This type of deposition also facilitates manufacture, and permits very precise control of the thickness of the fusible link.

After initial placement of the fusible link and the base copper onto the substrate or core, additional layers of a conductive metal are placed onto the terminal pads. These additional layers could be defined and placed onto these pads by photolithography and deposition techniques, respectively.

This fuse may be made by the following process. Shown in FIGS. 1 and 2 is a solid sheet 10 of an FR-4 epoxy with copper plating 12. The copper plating 12 and the FR-4 epoxy core 13 of this solid sheet 10 may best be seen in FIG. 2. This copper-plated FR-4 epoxy sheet 10 is available from Allied Signal Lamine Systems, Hoosick Falls, N.Y., as Part No. 0200BED130C1/C1GFN0200 C1/C1A2C. Although FR-4 epoxy is a preferred material, other suitable materials include any material that is compatible with, i.e., of a chemically, physically and structurally similar nature to, the materials from which PC boards are made. Thus, another suitable material for this solid sheet 10 is polyamide. FR-4 epoxy and polyamide are among the class of materials having physical properties that are nearly identical with the standard substrate material used in the PC board industry. As a result, the fuse of the invention and the PC board to which that fuse is secured have extremely well-matched thermal and mechanical properties. The substrate of the fuse of the present invention also provides desired arc-tracking characteristics, and simultaneously exhibits sufficient mechanical flexibility to remain intact when exposed to the rapid release of energy associated with arcing.

In the next step of the manufacture of the fuses of the present invention, the copper plating 12 is etched away from the solid sheet 10 by a conventional etching process. In this conventional etching process, the copper is etched away from the substrate by a ferric chloride solution.

Although it will be understood that after completion of this step, all of the copper layer 12 of FIG. 2 is etched away from FR-4 epoxy core 13 of this solid sheet 10, the remaining epoxy core 13 of this FR-4 epoxy sheet 10 is different from a "clean" sheet of FR-4 epoxy that had not initially been treated with a copper layer. In particular, a chemically etched surface treatment remains on the surface of the epoxy core 13 after the copper layer 12 has been removed by etching. This treated surface of the epoxy core 13 is more receptive to subsequent operations that are necessary in the manufacture of the present surface-mounted subminiature fuse.

The FR-4 epoxy sheet 10 having this treated, copper-free surface is then routed or punched to create slots 14 along quadrants of the sheet 10, as may be seen in FIG. 3. Dotted lines visually separate these four quadrants in FIG. 3. The

width W of the slots 14 (FIG. 4) is about 0.0625 inches. The length L of each of the slots 14 (FIG. 3) is approximately 5.125 inches.

When the routing or punching has been completed, the etched and routed or punched sheet 10 shown in FIG. 3 is again plated with copper. This reapplication of copper occurs through the immersion of the etched and routed sheet of FIG. 3 into an electro less copper plating bath. This method of copper plating is well-known in the art.

This copper plating step results in the placement of a copper layer having a uniform thickness along each of the exposed surfaces of the sheet 10. For example, as may be seen in FIG. 4, the copper plating 18 resulting from this step covers both (1) the flat, upper surfaces 22 of the sheet 10; and (2) the vertical, interstitial regions 16 that define at least a portion of the slots 14. These interstitial regions 16 must be copper-plated because they will ultimately form a portion of the terminal pads of the final fuse.

The uniform thickness of the copper plating will depend upon the ultimate needs of the user. Particularly, as may be seen in FIG. 4, for a fuse intended to open at  $1/16$  ampere, the copper plating 18 has a thickness of 2,500 Angstroms. For a fuse intended to open at 5 amperes, the copper plating 18 has a thickness of approximately 75,000 Angstroms.

After plating has been completed, to arrive at the copper-plated structure of FIG. 4, the entire exposed surface of this structure is covered with a so-called photoresist polymer.

An otherwise clear mask is placed over the replated copper sheet 20 after it has been covered with the photoresist. Square panels are a part of, and are evenly spaced across, this clear mask. These square panels are made of an UV light-opaque substance, and are of a size corresponding to the size of the rectangle 30 shown in FIG. 5. Essentially, by placing this mask having these panels onto the replated copper sheet 20, several portions of the flat, upward-facing surfaces 22 of the replated copper sheet 20 are effectively shielded from the effects of UV light.

It will be understood from the following discussion that these square panels will essentially define the shapes and sizes of the so-called fusible link 42 and the wide terminal areas 60 and 62 on the upper portion 22 of the fuse. The fusible link 42 is in electrical communication with the wide terminal areas 60 and 62. It will be appreciated that the width, length and shape of both the fusible link 42 and these wide terminal areas 60 and 62 may be altered by changing the size and shape of these UV light-opaque panels.

Additionally, the backside of the sheet is covered with a photoresist material and an otherwise clear mask is placed over the replated copper sheet 20 after it has been covered with the photoresist. A rectangular panel is a part of this clear mask. The rectangular panels are made of a UV light-opaque substance, and are of a size corresponding to the size of the panel 28 shown in FIG. 6. Essentially, by placing this mask having these panels onto the replated copper sheet 20, several strips of the flat, downward-facing surfaces 28 of the replated copper sheet 20 are effectively shielded from the effects of the UV light.

The rectangular panels will essentially define the shapes and sizes of the wide terminal areas 34 and 36 on the lower middle portion 28 of the underside of the strip 26.

The copper plating from a portion of the underside of a strip 26 is defined by a photoresist mask. Particularly, the copper plating from the lower, middle portion 28 of the underside of the strip 26 is removed. The lower, middle portion 28 of the underside of the strip 26 is that part of the strip along a line immediately beneath the areas 30 of clear

epoxy. A perspective view of this section of this repleted sheet 20 is shown in FIG. 6.

The entire repleted, photoresist-covered sheet 20, i.e., the top, bottom and sides of that sheet, is then subjected to UV light. The repleted sheet 20 is subjected to the UV light for a time sufficient to ensure curing of all of the photoresist that is not covered by the square panels and rectangular strips of the masks. Thereafter, the masks containing these square panels and rectangular strips are removed from the repleted sheet 20. The photoresist that was formerly below these square panels remains uncured. This uncured photoresist is still in a liquid form and, thus, may be washed from the repleted sheet 20.

The cured photoresist on the remainder of the repleted sheet 20 provides protection against the next step in the process. Particularly, the cured photoresist prevents the removal of copper beneath those areas of cured photoresist. The regions formerly below the square panels have no cured photoresist and no such protection. Thus, the copper from those regions can be removed by etching. This etching is performed with a ferric chloride solution.

After the copper has been removed, as may be seen in FIGS. 5 and 6, the regions formerly below the square panels and the rectangular strips of the mask are not covered at all. Rather, those regions now comprise areas 28 and 30 of clear epoxy.

The repleted sheet 20 is then placed in a chemical bath to remove all of the remaining cured photoresist from the previously cured areas of that sheet 20.

For the purposes of this specification, the portion of the sheet 20 between adjacent slots 14 is known as a strip 26. This strip has a dimension D as shown in FIG. 4 which defines the length of the device. After completion of several of the operations described in this specification, this strip 26 will ultimately be cut into a plurality of pieces, and each of these pieces becomes a fuse in accordance with the invention.

As may also be seen from FIG. 6, the underside 32 of the strip 26 has regions along its periphery which still include copper plating. These peripheral regions 34 and 36 of the underside 32 of the strip 26 form portions of the pads. These pads will ultimately serve as the means for securing the entire, finished fuse to the PC board.

FIG. 7 is a perspective view of the top-side 38 of the strips 26 of FIG. 6. Directly opposite and coinciding with the lower, middle portions 28 of these strips 26 are linear regions 40 on this top-side 38. These linear regions 40 are defined by the dotted lines of FIG. 7.

FIG. 7 is to be referred to in connection with the next step in the manufacture of the invention. In this next step, a photoresist polymer is placed along each of the linear regions 40 of the top side 38 of the strips 26. Through the covering of these linear regions 40, photoresist polymer is also placed along the relatively thin portions which will comprise the fusible links 42. These fusible links 42 are made of a conductive metal, here copper. The photoresist polymer is then treated with UV light, resulting in a curing of the polymer onto linear region 40 and its fusible links 42.

As a result of the curing of this polymer onto the linear region 40 and its fusible links 42, metal will not adhere to this linear region 40 when the strip 26 is dipped into an electrolytic bath containing a metal for plating purposes.

In addition, as explained above, the middle portion 28 of the underside 32 of the strip 26 will also not be subject to plating when the strip 26 is dipped into the electrolytic

plating bath. Copper metal previously covering this metal portion had been removed, revealing the bare epoxy that forms the base of the sheet 20. Metal will not adhere to or plate onto this bare epoxy using an electrolytic plating process.

The entire strip 26 is dipped into an electrolytic copper plating bath and then an electrolytic nickel plating bath. As a result, as may be seen in FIG. 8, copper 46 and nickel layers 48 are deposited on the base copper layer 44. After deposition of these copper 46 and nickel layers 48, the cured photoresist polymer on the linear region 40, including the photoresist polymer on the fusible links 42, is removed from that region 40.

Photoresist polymer is then immediately reapplied along the entire linear region 40. As may be seen in FIG. 9, however, a portion 50 at the center of the fusible link 42 is masked with a UV light-opaque substance. The entire linear region 40 is then subjected to UV light, with the result that curing of the photoresist polymer occurs on all of that region, except for the masked central portion 50 of the fusible link 42. The mask is removed from the central portion 50 of the fusible link, and the strip is rinsed. As a result of this rinsing, the uncured photoresist above the central portion 50 of the fusible link 42 is removed from the fusible link. The cured photoresist along the remainder of the linear region 40, however, remains.

Plating of metal will not occur on the portion of the strip 26 covered by the cured photoresist. Because of the absence of the photoresist from the central portion 50 of the fusible link 42, however, metal may be plated onto this central portion 50.

When the strip shown in FIG. 9 is dipped into an electrolytic tin plating bath, a tin layer 52 (FIG. 10) is overlain over the copper 46 and nickel layers 48. A tin spot 54 is also deposited onto the surface of the fusible link 42, i.e., essentially placed by an electrolytic plating process onto the central portion 50 of the fusible link 42. This electrolytic plating process is essentially a thin film deposition process. It will be understood, however, that this tin may also be added to the surface of the fusible link 42 by a Photolithographic process or by means of a physical vapor deposition process, such as sputtering or evaporation in a high vacuum deposition chamber.

This spot 54 is comprised of a second conductive metal, i.e., tin, that is dissimilar to the copper metal of the fusible link 42. This second conductive metal in the form of the tin spot 54 is deposited onto the fusible link 42 in the form of a rectangle.

The tin spot 54 on the fusible link 42 provides that link 42 with certain advantages. First, the tin spot 54 melts upon current overload conditions, creating a fusible link 42 that becomes a tin-copper alloy. This tin-copper alloy results in a fusible link 42 having a lower melting temperature than either the tin or copper alone. The lower melting temperature reduces the operating temperature of the fuse device of the invention, and this results in improved performance of the device.

Although tin is deposited on the copper fusible link 42 in this example, it will be understood by those skilled in the art that other conductive metals may be placed on the fusible link 42 to lower its melting temperature, and that the fusible link 42 itself may be made of conductive metals other than copper. In addition, the tin or other metal deposited on the fusible link 42 need not be of a rectangular shape, but can take on any number of additional configurations.

The second conductive metal may be placed in a notched section of the link, or in holes or voids in that link. Parallel

fuse links are also possible. As a result of this flexibility, specific electrical characteristics can be engineered into the fuse to meet varying needs of the ultimate user.

As indicated above, one of the possible fusible link configurations is a serpentine configuration. By using a serpentine configuration, the effective length of the fusible link may be increased, even though the distance between the terminals at the opposite ends of that link remain the same. In this way, a serpentine configuration provides for a longer fusible link without increasing the dimensions of the fuse itself.

The next step in the manufacture of the device of the invention is the placement, across the length of the entire top portion 38 of the strip 26, of a novel protective layer 56 (FIGS. 11 and 12). This protective layer 56 is the second subassembly of the present fuse, and forms a relatively tight seal over the top portion 38 of the strip 26, including the fusible link 42. In this way, the protective layer 56 inhibits corrosion of the fusible links 42 during their useful lives. The protective layer 56 also provides protection from oxidation and impacts during attachment to the PC board. The protective layer 56 of the present invention is advantageous over prior protective layers, in that the present protective layer does not extend beyond the dimensions of the peripheral regions 34 and 36 of the fuse.

This protective layer 56 helps to control the melting, ionization and arcing which occur in the fusible link 42 during current overload conditions. The protective layer 56 or cover coat material provides desired arc-quenching characteristics, especially important upon opening of the fusible link 42.

The novel protective layer 56 may be comprised of a polymer, preferably a photoimageable substance, such as DUPONT Pyralux® PC 2000 flexible photoimageable coverlay, or a photoimageable liquid. Other similar photoimageable materials are suitable for the invention.

The entire exposed surface of the structure of FIG. 10 is covered with a so-called photoimageable material, the novel conformal coating. There are at least two ways of placing this photoimageable material onto the structure of FIG. 10.

The first way is by a liquid photoimageable material (LPI) sprayed onto the structure of FIG. 10. This LPI is then subjected to a brief drying step, where it is tack-dried.

The second way is by a dry photoimageable material or photoimageable coverlay (PIC), such as a film, applied by vacuum lamination. This is vacuum laminated, and therefore needs no tack drying step.

In U.S. Pat. No. 5,552,757, no artwork is used to limit the extent of coverage of the conformal coating. In the present application, artwork is used to define the extent of coverage of the photoimageable conformal coating.

A distinct advantage of the present application over the teachings of U.S. Pat. No. 5,552,757 is its superior conformal coating height control. The use of the photoimageable material as the conformal coating results in a coating height that is only about 2.5% of the coating height of the conformal coating in the '757 patent. Particularly, in the '757 patent, the height of the conformal coating (56 in FIGS. 11 and 12 of the '757 patent) is approximately 20 mils. In the present FIGS. 11 and 12, the height of the conformal coating 56 is approximately 0.5 mils.

This provides the present invention with a significant advantage over the structure of the '757 patent. Because of the height of the conformal coating in the '757 patent, the side of that structure having the conformal coating must be

positioned facing upwardly. If one were to place the side having the conformal coating downwardly, i.e., facing the circuit board, the height of the coating would cause the terminals on this structure to be separated from the circuit board, preventing contact between the terminals and the circuit board. There is yet another disadvantage in the coating of the '757 patent. In the device of the '757 patent, it is possible that upon blowing of the fuse under current overload conditions, the molten metal from the fuse element can be spewed upwardly or outwardly. When this metal lands, it can contact other metallic elements on the PC board. As a result, these metallic elements can suffer from short circuits.

In contrast, the present invention has a very thin conformal coating, enabling the side of the surface mounted fuse with this coating to be placed downwardly, i.e., facing and in contact with the circuit board. As a result, the fusible link faces the PC board, rather than facing upwardly. Thus, upon blowing of the fuse link under current overload conditions, the downwardly-facing fuse link will not spew its molten metal upwardly, and will thus not endanger other sensitive metallic elements on the circuit board.

The thin conformal coating of the present invention, and its method of manufacture, provide another significant advantage. Particularly, the relatively thick conformal coating of the device of the '757 patent was subject to "wicking". This "wicking" phenomenon caused a portion of the coating to cover parts of the terminals of the '757 surface-mount fuse. The obvious result of this was to interfere with the electrical contact between the terminals and the corresponding mounting surface on the printed circuit board.

The "wicking" phenomena is avoided in the present invention, ensuring maximum contact between the terminals of the present surface-mount fuse and the mounting surface of the printed circuit board. "Wicking" is avoided both because of the minimal thickness of the conformal coating, and because the terminals are covered by artwork during manufacture.

As noted above, there are two methods of applying a photoimageable material. Both methods, the application of a liquid photoimageable (LPI) coating and a dry photoimageable coating, result in essentially the same finished product. Application of LPI Coating, as by Spraying

The entire exposed surface of the structure of FIG. 10 is covered with a so-called photoimageable material as a conformal coating. There are at least two ways of placing this photoimageable material onto the structure of FIG. 10. The first way is by spraying a liquid photoimageable material (LPI) onto the structure of FIG. 10.

The LPI is made by blending various components. A two part composition is blended. The first component of this two-part composition is made by Hysol, and is sold as HYSOL SR 8400 Liquid Photoimageable Material (LPI) solder resist. The second component of this two-part composition is also made by Hysol, and is sold as HYSOL solder resist catalyst. These two components are mixed in amounts of 85 parts LPI solder resist to 15 parts solder resist catalyst.

After blending, the composition is somewhat viscous, having the consistency of a gelatin. In order to facilitate the spraying of this composition onto the structure of FIG. 10, it is preferred that a solvent be added. The preferred solvent for the present invention is UCAR PM solvent, which is methoxy 2-propanol, packaged by Produceos Chemical Co. of Batavia, Ill. About 0.4 to 0.5 gram of UCAR PM solvent is added to each gram of the viscous composition made from the HYSOL solder resist/solder resist catalyst.

This composition, diluted with the solvent, is now ready for spraying onto the structure of FIG. 10. It is here sprayed

only onto one side of the structure; however, the composition may also be sprayed onto both sides of the structure. Thereafter, the panel is placed into an oven at approximately 185 degrees C., and is held in that oven for from 30 to 45 minutes until the surface is "tack dry."

The tack dry panel is then removed from the oven, and artwork is then placed over the entire panel. The artwork covers sections of the panel with an opaque portion that prevents passage of ultraviolet rays. The opaque portion of the artwork covers the terminals.

The artwork-covered panel is then placed into an Accuprint AP-30-6000 Titan ultraviolet (UV) chamber. It is subjected to ultraviolet radiation at approximately 250 mJoules/cc for 45 seconds.

The panel is now removed from the UV chamber. The uncovered portions of the panel have been largely cured by the ultraviolet radiation. The portions of the panel beneath the opaque portion of the artwork, i.e., the terminals, remain uncured.

The uncured composition is ready for removal from the terminals of the panel, so that the metallization below the opaque portion will be exposed. The uncured composition is removed by processing through a Coates ASI conveyorized system utilizing pressurized nozzles dispensing a solution of 1½% sodium carbonate in water. The panel is moved through this dilute sodium carbonate solution at 1.5 feet per minute, and is then rinsed in a pure water bath. From this water bath, the panel exits the unit.

The wet panel is now removed from the water bath. A final step both dries the panel and completely cures the liquid photoimageable material. In this step, the panel is placed into an oven at 120 to 150 degrees C. for approximately one (1) hour.

#### Application of Dry Photoimageable Overlay (PIC) Material, as by Vacuum

As an alternative to the application of a liquid photoimageable material, a dry photoimageable material may be applied. As noted above, the entire exposed surface of the structure of FIG. 10 may be covered with a liquid photoimageable material 56 as a conformal coating. The alternative, second way of applying the photoimageable material as a conformal coating is by the application of a dry photoimageable material adhered by vacuum lamination.

As noted above, the LPI was made by blending a two part composition. In contrast, the dry photoimageable material is obtained in a ready-to-use form. The most preferred dry photoimageable material is obtained from DuPont Electronics Materials, 14 T.W. Alexander Drive, Research Triangle Park, N.C. 27709-4425. It is sold under the registered trademark Pyralux® PC 2000. The product code for the most preferred Pyralux® flexible composite is PC2010, which has a thickness of 25 microns (1.0 mils).

A sheet of the Pyralux® PC2010 is overlaid onto the only one side of the structure shown in FIG. 10, although it may be placed on both sides. The composite structure is then placed into a Vacrel 100 vacuum laminator, set at about 70-83 degrees C., and that structure remains in the vacuum chamber for a 30-60 second dwell time, with a slap down, or laminating, time of 5 to 10 seconds.

The panel is then removed from the vacuum chamber, and artwork is placed over the entire panel. The artwork covers sections of the panel with an opaque portion that prevents passage of ultraviolet rays. The artwork-covered panel is placed into an Accuprint AP-30-6000 Titan ultraviolet (UV) chamber. It is subjected to ultraviolet radiation at approximately 250 mJoules/cc for 45 seconds.

The panel is then removed from the UV chamber. The uncovered portions of the panel have been largely cured by

the ultraviolet radiation. The portions of the panel beneath the opaque portion of the artwork, i.e., the terminals, remain uncured.

The uncured photoimageable material from the flexible composite is ready for removal from the panel, so that the terminal metal below the opaque portion created by the artwork will be exposed. The uncured composition is removed by processing through a Coates ASI conveyorized system utilizing pressurized nozzles dispensing a solution of 1½% sodium carbonate in water. The panel is moved through this dilute sodium carbonate solution at 1.5 feet per minute, and is then rinsed in a pure water bath. From this water bath, the panel exits the unit.

A final step both dries the panel and completely cures the photoimageable material, i.e., the flexible composite. In this step, the panel is placed into an oven at 120 to 150 degrees C. for approximately one (1) hour.

Although a colorless, clear photoimageable material is aesthetically pleasing, alternative types of materials may be used. For example, colored, clear materials may be used. These materials may be used on the bottom and the top of the surface-mount fuse. These colored photoimageable materials may be simply manufactured by the addition of a dye to a clear photoimageable material. Color coding may be accomplished through the use of these colored photoimageable materials. In other words, different colors of photoimageable materials can correspond to different amperages, providing the user with a ready means of determining the amperage of any given fuse. The transparency of both of these coatings permit the user to visually inspect the fusible link 42 prior to installation, and during use in the electronic device in which the fuse is used.

The use of this protective layer 56 has significant advantages over the prior art, including the prior art, so-called, "capping" method. Due to the placement of the protective layer 56 over the entire top portion 38 of the fuse body, the location of the protective layer relative to the location of the fusible link 42 is not critical.

Whether the photoimageable material has been applied as a liquid or solid, the strips 26 are then ready for a so-called dicing operation, which separates those strips 26 into individual fuses. In this dicing operation, a diamond saw or the like is used to cut the strips 26 along parallel planes 57 (FIG. 11) into individual thin film surface-mounted fuses 58 (FIG. 12). The cuts bisect the wide terminal areas 60 and 62 of the thin film copper patterns. These wide terminal areas 60 and 62 appear on either side of the fusible link 42.

This cutting operation completes the manufacture of the thin film surface-mounted fuse 58 (FIG. 12) of the present invention.

Fuses in accordance with this invention are rated at voltages and amperages greater than the ratings of prior art devices. Tests have indicated that fuses in accordance with this invention would have a fuse voltage rating of 60 volts AC, and a fuse amperage rating of between  $\frac{1}{16}$  ampere and 5 amperes. Even though the fuses in accordance with this invention can protect circuits over a broad range of amperage ratings, the actual physical size of these fuses remains constant.

In summary, the fuse of the present invention exhibits improved control of fusing characteristics by regulating voltage drops across the fusible link 42. Consistent clearing times are ensured by (1) the ability to control, through deposition and photolithography processes, the dimensions and shapes of the fusible link 42 and wide terminals 60 and 62; and (2) proper selection of the materials of the fusible link 42. Restriking tendencies are minimized by selection of an optimized material for the substrate 13 and protective layer 56.

**11**

Another preferred embodiment comprises using a slightly different first subassembly as the basis of the invention. This different first subassembly includes holes or bores **14**, and is described in U.S. patent application Ser. No. 08/472,563, filed on Jun. 7, 1995. The pertinent part of this specification which describes this different first subassembly and its method of manufacture appears at pages 12-28 of the specification, which is hereby incorporated by reference. The Figures illustrating this embodiment appear in the application as FIGS. **4-12**, which are also incorporated herein by reference.

Specific embodiments have been illustrated and described. The scope of protection is limited only by the scope of the accompanying Claims.

What I claim is:

**1.** A thin film fuse for mounting on a surface, said fuse comprising two material subassemblies:

a. the first subassembly comprising a fusible link, its supporting substrate and terminal pads; and

**12**

b. the second subassembly consisting of a single layer of photoimageable material as a conformal coating that overlies and contacts the fusible link, the photoimageable material having a thickness such that the height of the conformal coating will not prevent the mounting of the fuse on the surface with the fusible link facing either downwardly or upwardly with respect to the surface.

**2.** The surface-mount fuse of claim **1**, wherein said photoimageable material is applied as a liquid.

**3.** The surface-mount fuse of claim **2** wherein said photoimageable material is clear and colored.

**4.** The surface-mount fuse of claim **1**, wherein said photoimageable material is applied as a solid.

**5.** The surface-mount fuse of claim **4**, wherein said solid photoimageable material is a film.

**6.** The surface-mount fuse of claim **1** wherein said photoimageable material is clear and colored.

\* \* \* \* \*